

March 2, 1971

E. LAND

3,567,442

NOVEL PHOTOGRAPHIC PRODUCTS AND PROCESSES

Original Filed Dec. 9, 1959



FIG. 1



FIG. 2



FIG. 3

INVENTOR

Edwin H. Land

BY

Brown and Mikulka

ATTORNEYS

**1****3,567,442**  
**NOVEL PHOTOGRAPHIC PRODUCTS AND PROCESSES**

Edwin Land, Cambridge, Mass., assignor to Polaroid Corporation, Cambridge, Mass.  
Continuation of application Ser. No. 858,454, Dec. 9, 1959. This application Mar. 10, 1967, Ser. No. 622,133  
Int. Cl. G03c 5/54

U.S. Cl. 96—29

3 Claims

**ABSTRACT OF THE DISCLOSURE**

The present invention is directed to a silver diffusion transfer photographic process print-receiving element which comprises a common support carrying on one surface a plurality of layers each of which comprises metallic sulfide, metallic selenide, colloidal metal, thiooxalate or thioacetamide silver precipitating agents disposed in a gelatin, deacetylated chitin or silica matrix wherein each such layer comprises a substantially constant concentration of silver precipitating agent per unit area, and a decreasing concentration, layer-wise, in the direction of the support; and to photographic silver diffusion transfer processes employing such print receiving element.

This application is a continuation of my copending U.S. application Ser. No. 858,454, filed Dec. 9, 1959.

This invention relates to photographic products and processes for the fabrication and utilization of said products and more particularly to photographic products useful in diffusion-transfer processes wherein a latent image contained in an exposed silver halide emulsion is developed therein and a soluble silver complex, obtained by reaction of the undeveloped silver halide of said emulsion with an appropriate silver halide solvent, is transferred from said emulsion to an image-receiving element to provide therein a reversed positive silver image of the latent image, and to processes for the fabrication of said products.

A principal object of the present invention is to provide transfer processes for the aforementioned type and products for utilization therein whereby positive prints are produced exhibiting enhanced quality and stability.

A further object of the present invention is to provide improved products particularly useful in the aforementioned diffusion-transfer processes as print-receiving elements, each of said products comprising a multilayer image-receiving stratum, wherein each layer of said stratum contains a progressively increasing concentration of silver precipitating nuclei in respect to the concentration of said nuclei contained in adjacent layers, positioned less distant from the surface of the print-receiving element in contact with a silver halide transferring medium, to thereby produce dense positive silver images of excellent pictorial quality and improved stability.

A still further object of the present invention is to provide transfer processes of the aforementioned type and products for utilization therein whereby silvering, due to surface precipitation of elemental silver on a print-receiving element, is avoided.

Other objects of the invention will in part be obvious and will in part appear hereinafter.

The invention accordingly comprises the several steps and relation and order of one or more of such steps with respect to each of the others, and the product possessing the features, properties and relation of elements which

**2**

are exemplified in the following detailed disclosure, and the scope of the application of which will be indicated in the claims.

For a fuller understanding of the nature and objects of the invention, reference should be had to the following 5 detailed description taken in connection with the accompanying drawing wherein:

FIG. 1 is a diagrammatic enlarged cross-sectional view illustrating the association of elements during one stage of the performance of a transfer process and showing as one of the elements an embodiment of the novel print-receiving elements of the present invention, the thickness of the various materials being exaggerated;

FIG. 2 is a diagrammatic enlarged cross-sectional view of one form of the novel print-receiving elements of the 10 present invention; and

FIG. 3 is a diagrammatic enlarged cross-sectional view illustrating the association of elements during one stage of the performance of another transfer process.

The present invention comprehends improved diffusion-transfer reversal processes and products of the type whereby a positive print is obtained in a single step by suitably treating a silver halide emulsion containing a latent image with a processing liquid. Preferably, the processing liquid 20 is in a viscous condition and is spread in a thin film between the photosensitive element comprising a silver halide emulsion and a multilayer image-receiving element containing varying concentrations of silver precipitants. The processing composition develops the latent image in 25 the emulsion and forms a soluble complex, for example, a thiosulfate or a thiocyanate complex, with undeveloped silver halide. This soluble silver complex is transferred, at least in part, by imbibition, to the print-receiving element and the silver component thereof is precipitated in 30 the multilayer image-receiving stratum of the print-receiving element to provide a reversed, positive silver image of the latent image therein.

It has been proposed to use in the formation of silver transfer prints by the aforementioned processes such materials as, for example, the metallic sulfides and selenides, thiooxalates and thioacetamides, disclosed in U.S. Pat. No. 2,647,056, issued July 28, 1953 to Edwin H. Land. Examples of silver precipitating agents or nuclei of the preferred type are the so-called "heavy metal" sulfides of 40 zinc, chromium, gallium, iron, cadmium, cobalt, nickel, lead, antimony, bismuth, silver, cerium, arsenic, copper and rhodium and the selenides of lead, zinc, antimony and nickel. Other precipitating agents have been proposed such as, for example, the colloidal metals and specifically 45 colloidal silver. The use of silver precipitating agents to aid in the reduction and precipitation of metallic silver from silver complex ions in the presence of a silver halide developing agent in photographic diffusion-transfer reversal processes is well known to the art and does not 50 per se constitute a feature of this invention.

Further, it has been proposed to use in the formation of silver transfer prints by the previously-mentioned processes certain special matrices in which the silver precipitating agent is so dispersed as to effect a controlled 55 precipitation of the soluble silver complex, the chosen matrix serving to receive and suitably aggregate the precipitated silver to produce therein positive images. Preferably the silver precipitating agents are dispersed in a suitable matrix formed of particles, preferably colloidal in size, of a chemically inert, absorbent material. It is preferable that these particles have a relatively low coefficient of absorption for light as compared to silver and satisfactory examples of materials of this type are: colloidal

silica, such as silica aerogel, fuller's earth, diatomaceous earth, kieselguhr, wood flour, infusorial earth, bentonite, filter aids such as Celite and Super-Floss (trade names of Johns-Manville Sales Corp., New York, N.Y., for diatomaceous earth filtration aids), and finely powdered glass, talc, mica or zinc oxide. The use of a chemically inert, absorbent matrix to aid in the precipitation of the soluble silver complex in photographic diffusion-transfer reversal processes is well known to the art and does not per se constitute a feature of this invention.

According to the present invention, the precipitation and aggregation of silver obtained by using silver precipitating agents, including the aforementioned materials, is greatly improved and expedited by providing a print-receiving element having a plurality of layers containing a varying concentration of silver precipitating agents, especially wherein the concentration of silver precipitating nuclei progressively increases as the distance of the respective layers from the external surface of the image-receiving stratum increases.

It will be recognized that the concentration of silver precipitating nuclei within one or more layers may remain constant or vary, that is, vary randomly or according to a prearranged distribution. In addition, the matrix of each layer may comprise, where desired, a single component or a mixture of components, and two or more layers may comprise different matrices.

The novel print-receiving element is preferably fabricated by successively applying to a suitable support the respective silver precipitating nuclei-containing layers. The respective layers are preferably dried prior to successive coating operations. The support may be formed of a material such as, for example, paper, regenerated cellulose, polyvinyl alcohol, cellulose ethers such as methyl cellulose, ethyl cellulose, or their derivatives, and other natural and synthetic gums and resins which will form continuous films and which are relatively stable, mechanically, in the presence of water and alkali. The supporting sheets are preferably opaque when a reflection print is desired and transparent when a transparency is desired.

As previously noted, it is preferable that the respective layers be dried prior to successive coating operations. However, it must be noted that even though the layers are deposited under dry conditions the interface between contiguous layers may dissipate, particularly where a common matrix material is used for the several layers.

One method of preparing the respective silver precipitating agent-containing layers may comprise forming a dispersion of silver precipitating agents by vacuum depositing, as for example, by cathode sputtering, an appropriate silver precipitating agent on a suitable matrix and blending the resulting product in a coating solvent. Processes of the aforementioned type are disclosed in the copending U.S. application of Edwin H. Land, Ser. No. 705,845, filed Dec. 30, 1957, abandoned and replaced by Ser. No. 249,922, filed Jan. 7, 1963, now U.S. Pat. No. 3,295,972, issued Jan. 3, 1967. The coating compositions containing the desired concentration of silver precipitating agents are prepared by dilution of the aforementioned blended product. Next, the respective coating compositions comprising progressively decreasing concentrations of silver precipitating agents are successively coated on a suitable support. As previously mentioned, it is preferred that each successive layer be dried prior to succeeding coating operations.

An illustrative process for forming the novel print-receiving elements of the present invention is set out below.

A coating formulation is prepared by evaporating 10 parts of silver onto 400 parts of twenty mesh carboxymethyl cellulose powder. 5 parts of the resultant product are dissolved in 100 parts of an aqueous gelatin composition containing 2% of gelatin and 2% deacetylated chitin. (Image-receiving layers containing deacetylated chitin

are disclosed and claimed in U.S. Pat. No. 3,087,815 issued Apr. 30, 1963 in the name of William H. Ryan and Elizabeth L. Yankowski.) A support comprising a polyvinyl butyral-coated baryta paper is coated with the aforementioned formulation. After the coating has dried, a second layer comprising the aforementioned formulation diluted in the ratio of 1 cc. to 9 cc. with the aforementioned gelatin-deacetylated chitin composition is coated on the exposed surface of the initial coating and dried.

Particularly desirable results are obtained when the silver precipitating agents in the image-receiving layer are disposed in a matrix comprising a macroscopically continuous stratum comprising submacroscopic agglomerates of minute particles of a suitable water-insoluble, inorganic, preferably siliceous material, such, for example, as silica aerogel. Suitable matrices of this type are disclosed in U.S. Pat. No. 2,698,237.

Other techniques for incorporating a silver precipitating agent, such as dissolving said agent in a solution of 20 the matrix-forming material, may also be employed.

It will be recognized that the silver-receptive stratum of the present invention is so constituted as to provide an unusually vigorous elemental silver precipitating environment which causes the elemental silver deposited 25 therein, in comparison with the amount of silver developed in the silver halide photosensitive layer, to possess very high covering power, that is, opacity for given mass of reduced silver.

Especially suitable as silver precipitating agents are the 30 metallic sulfides and selenides, these terms being understood to include the selenosulfides, the polysulfides, and the polyselenides. Preferred in this group are the so-called "heavy metal sulfides" previously noted. For best results it is preferred to employ sulfides whose solubility 35 products in an aqueous medium at approximately 20° C. vary between  $10^{-23}$  and  $10^{-30}$  and especially the salts of zinc, cadmium and lead. Also suitable as precipitating agents are heavy metals such as silver, gold, platinum, palladium, and mercury, and in this category the noble 40 metals are preferred and are preferably provided in the matrix as colloidal particles. The salts of these heavy metals, preferably the simple inorganic and readily reducible salts such as silver nitrate, gold chloride and gold nitrate, are also useful as silver precipitating agents. 45 In some instances, the metals are introduced into the matrices as salts and then reduced in situ prior to the use of the reception material in the silver transfer process to give a layer whose silver precipitating agent is a colloidal metal. Where the salts are relatively light- or heat-sensitive, this reduction may be accomplished simply by exposing the silver precipitating layer to diffused light 50 or to heat. Still other satisfactory silver precipitating agents are certain of the thio compounds, for example, dithiooxalate and its lead and zinc complexes, potassium 55 dithiooxalate and the lead and nickel complexes thereof, and thioacetamide. The silver precipitating agents as noted above are provided in highly dispersed condition, preferably as colloidal particles.

Where the silver precipitating agent is one or more of 60 the heavy metal sulfides or selenides, it is preferable to prevent the diffusion and wandering of the sulfide or selenide ions, as the case may be, by also including, in the silver precipitating layers or in separate layers closely adjacent thereto, at least one metallic salt which is substantially more soluble in the processing agent than the heavy metal sulfide or selenide used as the silver precipitating agent and which is irreducible in the processing agent. This more soluble salt has, as its cation, a metal whose ion 65 forms sulfides or selenides which are difficultly soluble in the processing agent and which give up their sulfide or selenide ions to silver by displacement. Accordingly, in the presence of sulfide or selenide ions the metal ions of the more soluble salts have the effect of immediately precipitating the sulfide or selenide ions from solution. 70 These more soluble or ion-capturing salts may be either

soluble salts of any of the following metals: cadmium, cerium (ous), cobalt (ous), iron, lead, nickel, manganese, thorium, and tin. Satisfactory soluble and stable salts of the above metals may be found, for example, among the following groups of salts: the acetates, the nitrates, the borates, the chlorides, the sulfates, the hydroxides, the formates, the citrates, and the dithionates. The acetates and nitrates of zinc, cadmium, nickel, and lead are preferred. In general, it is also preferable to use the white or lightly colored salts although for certain special purposes the more darkly colored salts may be employed.

The previously mentioned ion-capturing salts may also serve a function of improving the stability of the positive print provided they possess, in addition to the aforementioned characteristics, the requisites specified in U.S. Pat. No. 2,584,030 issued to Edwin H. Land. For example, if the ion-capturing salt is a salt of a metal which slowly forms insoluble or slightly soluble metallic hydroxides with the hydroxyl ions in the alkaline processing liquid, it will suitably control the alkalinity of the print-receiving element to substantially, if not totally, prevent the formation of undesirable developer stains.

The use of the novel print-receiving elements of the present invention in the performance of a silver halide diffusion-transfer reversal process is illustrated diagrammatically in FIG. 1 wherein photosensitive element 12 comprises a support 10 and a photosensitive silver halide emulsion layer 11; a layer 13 comprises a relatively viscous processing composition; and print-receiving element 14 is one embodiment of the novel print-receiving elements of the present invention. As shown, the print-receiving element 14 comprises a suitable support 16 and a multilayer image-receiving stratum 15 with a varying concentration of silver precipitants.

Multilayer image-receiving stratum 15 is formed by successively coating a suitable support 16, for example of baryta paper, with a plurality of suspensions or sols containing progressively decreasing concentrations of silver precipitating nuclei in suitable matrices. Each successive layer is preferably permitted to dry preceding the coating of the succeeding layer.

Liquid layer 13 may be obtained by spreading the processing composition, for example, in a manner disclosed in U.S. Pat. No. 2,647,056, issued July 28, 1953 to Edwin H. Land. As disclosed in the aforementioned patent, a rupturable container may be positioned between the photosensitive element and the print-receiving element such that upon application of suitable pressure, for example by compression between a pair of opposed, suitably gapped rollers, said container fractures releasing a liquid processing composition in contact with the transfer surfaces of each of said elements. The processing composition may be one of the film-forming processing compositions disclosed in said patent. It may comprise, for example, a developing agent such as hydroquinone, an alkali such as sodium hydroxide, a silver halide complexing agent such as sodium thiosulfate, for forming a soluble silver complex with unexposed and undeveloped silver halide, and a high molecular weight, film-forming, thickening agent such as sodium carboxymethyl cellulose. All these materials are preferably in an aqueous solution. The various photographic reagents are preferably contained in solution in the processing liquid prior to the spreading thereof as layer 13. However, it must be noted that they may be in whole or in part added to the processing liquid as it is spread between elements 12 and 14, said reagents being so located on or adjacent to the surface of one or both of said elements as to be dissolved by or otherwise interacted with the liquid composition when the latter wets said elements.

An illustration of a process for forming a positive image, in which a silver halide transfer takes place and in which an embodiment of the novel products of the present invention is used as a print-receiving element in the performance of said process, is set out below.

A processing agent may be prepared which comprises:

|                                  | Grams |
|----------------------------------|-------|
| Water                            | 1860  |
| 5 Sodium carboxymethyl cellulose | 93    |
| Sodium sulfite                   | 78    |
| Sodium hydroxide                 | 74.6  |
| Sodium thiosulfate               | 14.5  |
| Citric acid                      | 38.5  |
| 10 Hydroquinone                  | 52    |

and is spread in a layer 13 between the coated surface of element 12 and a selectively exposed photosensitive silver halide emulsion 11. The lamination formed by the spreading of the processing agent in a layer 13 between elements 12 and 14 is kept intact for approximately one-half to one and one-half minutes, preferably one minute, and at the end of this time element 14 is stripped from element 12. Element 14, when so stripped, carries a reversed positive print in silver of the subject matter of the latent image in emulsion 11. The layer 13 of the processing composition preferably adheres to emulsion 11 and solidifies thereon.

Other materials may be substituted for those used in the foregoing process and the proportions may be varied to an appreciable extent. For example, the film-forming material in the processing agent which imparts the desired viscosity to the latter may be any of the high molecular weight polymers which are stable to alkali and which are soluble in aqueous alkaline solutions. For example, such other plastics as hydroxyethyl cellulose, polyvinyl alcohol, and the sodium salts of polymethacrylic acid and polyacrylic acid may be used. The plastic is preferably contained in the agent in sufficient quantity to impart to the composition a viscosity in excess of 1000 centipoises at a temperature of approximately 20° C. Preferably, the viscosity of the processing agent is of the order of 1000 to 200,000 centipoises.

Other developing agents may be used, for example, one of the following: p-aminophenol hydrochloride; bromohydroquinone; chlorohydroquinone; diaminophenol hydrochloride; diaminophenol dihydrochloride; tolhydroquinone; monomethyl-p-aminophenol sulfate; a mixture consisting by weight of  $\frac{1}{2}$  hydroquinone and  $\frac{1}{2}$  p-hydroxyphenylaminoacetic acid; and a mixture consisting by weight of  $\frac{1}{4}$  hydroquinone and  $\frac{3}{4}$  p-hydroxyphenylaminoacetic acid.

To form the soluble silver complex, such other complex-forming substances as sodium thiocyanate, ammonium thiocyanate and ammonia may be employed.

As illustrated diagrammatically in FIG. 3, another embodiment of the aforementioned diffusion-transfer processes comprises the relation of elements wherein spreader sheet 19 is associated with a rupturable container 20 holding at least a liquid photographic processing composition and a photosensitive silver halide emulsion layer 11 having in superposed relation thereto a novel print-receiving element 15 of the present invention on a support 16.

Upon compression of the spreader sheet 19, rupturable container 20 fractures, releasing its contents in a substantially uniform layer between spreader sheet 19 and a selectively exposed photosensitive silver halide emulsion layer 11. The processing composition permeates emulsion layer 11, developing the latent image contained therein. Substantially simultaneously, undeveloped silver halide forms a soluble silver complex, by means of a silver halide solvent, as a function of the point-to-point degree of exposure of said photosensitive emulsion. An imagewise distribution of soluble silver complex is formed in the unexposed areas of the photosensitive emulsion and transferred, at least in part, by imbibition, to print-receiving stratum 15, to form upon precipitation of elemental silver therein, a reversed positive silver image of the latent image. Subsequent to substantial precipitative deposition 75 of the image-forming elemental silver in stratum 15, photo-

sensitive emulsion 11 may be dissociated from print-receiving stratum 15, as by, for example, manual stripping.

In another form of the novel print-receiving elements of the present invention as illustrated in FIG. 2, it may be desirable to provide a coating on the silver precipitating layer 15 of a material, such as a plastic, more abrasion-resistant than the matrix of the precipitating nuclei-containing layers in order to protect the external surface of the image-receiving stratum. This overcoat of a plastic material may also serve as a layer which prevents adhesion of the film-forming processing composition 13 so that when element 17 is stripped from the photosensitive element 12, at the completion of processing, the film-forming processing composition layer 13 remains attached to photosensitive element 12. An embodiment of this construction is illustrated in FIG. 2 wherein layer 18 is a suitable support, layer 15 is a multilayer image-receiving stratum and there is applied over layer 15 a thin coating of an abrasion-resistant coating 18 which may be, for example, gum arabic, cellulose acetate hydrogen phthalate, polyvinyl alcohol, hydroxyethyl cellulose, methyl cellulose, ethyl cellulose, cellulose nitrate, sodium alginate, pectin, or poly-methacrylic acid. Layer 18 preferably has a thickness of the order of 1 to 3 microns, although if it is relatively water permeable, its thickness may be appreciably greater. Layer 18 may also contain one or more neutralizing agents which tend to improve the stability of the finished print. As previously noted, the protective coating 18 may further serve as a layer for minimizing the adhesion to the film-forming material of layer 13, particularly where said material is carboxymethyl cellulose.

Where desired, the solid film obtained from the film-forming processing fluid 13 may be caused to adhere to the print-receiving element 14 to provide a protective coating thereon or caused to adhere to photosensitive emulsion layer 11 rather than the print-receiving element, as for example, according to the procedures disclosed in U.S. Pat. No. 2,647,056, issued July 28, 1953 to Edwin H. Land.

In addition to varying the concentration of the silver precipitating agents, one may also vary the thicknesses of the individual layers of silver precipitating agents. It is also within the scope of this invention to utilize different silver precipitating agents in two or more of the layers and/or to utilize a mixture comprising two or more silver precipitating agents in one or more of the layers.

The positive print is subject to several sources of instability which stem, for example, from the oxidation of the developer in the highlights, the discoloration of some of the unexhausted chemical components in the positive print by exposure to visible and near visible radiation, the partial bleaching of the silver, and the interaction of the deposited silver with external sulfur and sulfides under conditions such that the structure of the precipitated silver is changed, usually to a yellow-to-brown form. This reduces the density and changes the tone of the positive transfer image. Diffusion-transfer processes utilizing the single layer print-receiving structures of the prior art inherently result in the deposition of a substantial quantity of the elemental silver precipitate on or adjacent to an exposed surface of the print-receiving element with the resultant proclivity of a substantial proportion of the positive image to adverse externally caused deterioration. In addition, the deposition of the elemental silver precipitate upon or in the surface area of the respective print-receiving elements provides an undesirable silvering effect. The novel print-receiving structures of the present disclosure alleviate the aforementioned undesirable effects in that they provide a reception element wherein the tendency of the silver halide complex is to provide a precipitate of elemental silver removed from the surface of said element.

In addition to the aforementioned increased stability afforded the positive image, the novel print-receiving struc-

tures of the present disclosure provide image formation exhibiting decreased granularity and graininess. The appearance of "graininess" in the transferred image is apparently not produced by the perception of individual submacroscopic grains of deposited elemental silver, but rather the optical impression of non-uniformity produced as a result of pattern effects which themselves appear to result from the irregular distribution of the elemental silver grains. When, as a result of the irregularity of the disposition of silver grains, a substantial number of the respective grains are deposited in close proximity, the optical effect is that of aggregation or clumping and, conversely, a deficiency in the concentration of deposited grains per unit area reflects incomplete image formation and definition. Inasmuch as the print-receiving structures of the present invention provide a vastly increased control of the elemental silver precipitation as well as the distribution of the precipitating sites in the image-receiving stratum, the aforementioned effects apparently due at least in part to random distribution of silver precipitate in prior art structures are avoided.

Further, the novel print-receiving structures disclosed herein provide increased resolving power, sharpness, density, contrast, covering power, and intensification resulting from an increased three-dimensional array of elemental silver precipitates per unit of viewed surface area.

The novel print-receiving elements of this invention provide several other advantages. They are more stable during storage prior to use. The images formed therein do not exhibit image "rub-off," which may occur where the image silver is precipitated on or close to the surface of the print-receiving element. In addition, the use of layers of varying concentrations of silver precipitants makes it possible to selectively encourage the characteristics of the toe or shoulder portions of the characteristic curve of the image. This, in turn, permits the formation of images with characteristic curves which are smooth, long, straight-line curves, thereby facilitating true copying of the resulting silver transfer images, as well as of other images.

Since certain changes may be made in the above products and processes without departing from the scope of the invention herein involved, it is intended that all matter contained in the above description or shown in the accompanying drawing shall be interpreted as illustrative ad not in a limiting sense.

What is claimed is:

1. In a process of forming a transfer image in silver which comprises the steps of developing an exposed silver halide emulsion with a processing composition comprising a silver halide developing agent and a silver halide solvent, forming an imagewise distribution of soluble silver complex in unexposed areas of said emulsion as a function of the point-to-point degree of exposure thereof, transferring from said emulsion, at least in part, by imbibition, said imagewise distribution of soluble silver complex to a print-receiving element in superposed relationship with said emulsion so as to receive a depth-wise diffusion of said imagewise distribution and providing thereby a silver transfer image, and separating said print-receiving element from its superposed relationship with said emulsion subsequent to substantial transfer image formation, the improvement which comprises providing a visible silver transfer image of improved stability comprising image silver precipitated in each of at least two contiguous layers by transferring said imagewise distribution of said soluble silver complex to a preformed substantially photoinsensitive print-receiving element comprising a common support having on one surface thereof a plurality of contiguous layers, each of said layers comprising the same solid matrix selected from the group consisting of gelatin, deacetylated chitin and a macroscopically continuous matrix comprising submacroscopic agglomerates of minute particles of water-insoluble, inorganic, chemically inert and absorbent silica matrices and an effective concentration of the same silver precipitating agent selected

from the group consisting of metallic sulfide, metallic selenide, colloidal metal, thiooxalate and thioacetamide silver precipitating agents adapted to effect precipitation of said soluble silver complex, wherein each layer of said plurality of layers comprises a substantially constant concentration of said agent, per unit area, within said layer and a decreasing concentration of silver precipitating agent, layerwise, as the distance of the respective layer from the common support increases, and said silver halide emulsion, in superposed relationship, is in superposition with the layer of said plurality of layers positioned most distal from support during said transfer of soluble silver complex from unexposed areas of said silver halide emulsion to said print-receiving element and said print-receiving element including said plurality of contiguous layers is separated from said superposed relationship with said emulsion subsequent to substantial transfer image formation.

2. As a photographic product, a substantially photoinsensitive diffusion transfer print-receiving element which comprises a common support having on one surface a plurality of contiguous layers, each of said layers including, dispersed in the same matrix selected from the group consisting of gelatin, deacetylated chitin and a macroscopically continuous matrix comprising submacroscopic agglomerates of minute particles of water-insoluble, chemically inert and absorbent silica matrices, a substantially constant concentration of the same silver precipitating agent selected from the group consisting of metallic sulfide, metallic selenide, colloidal metal, thiooxalate, and

thioacetamide silver precipitating agents, per unit area, within said layer, and a decreasing concentration of said silver precipitating agent, layerwise, as the distance of the respective layer from the common support increases effective to provide a visible silver transfer image comprising image silver precipitated in each of at least two said contiguous layers.

3. As a photographic product, a substantially photoinsensitive diffusion transfer print-receiving element which 10 comprises baryta paper carrying on one surface thereof, in order, first and second polymeric layers each comprising deacetylated chitin and gelatin and containing, as a silver precipitating agent, a substantially constant concentration of silver, said second polymeric layer containing 15 said silver at a concentration per unit area of about one-ninth of the concentration per unit area contained in said first polymeric layer next adjacent said surface of said baryta paper.

#### References Cited

##### UNITED STATES PATENTS

|           |         |             |       |       |
|-----------|---------|-------------|-------|-------|
| 2,563,342 | 8/1951  | Land        | ----- | 95—6  |
| 2,774,667 | 12/1956 | Land et al. | ----- | 96—29 |
| 3,313,625 | 4/1967  | Ryan        | ----- | 96—76 |

25 NORMAN G. TORCHIN, Primary Examiner

J. GOODROW, Assistant Examiner

U.S. Cl. X.R.

30 96—76